

## 1

3,558,490

### STYRYL PHOSPHORODITHIOATE ESTERS TO BE USED AS ANTIOXIDANTS IN LUBRICATING OIL

Warren Lowe, El Cerrito, Calif., assignor to Chevron Research Company, San Francisco, Calif., a corporation of Delaware  
No Drawing. Filed May 31, 1968, Ser. No. 733,310  
Int. Cl. C10m 1/48, 3/42  
U.S. Cl. 252—46.6

6 Claims

#### ABSTRACT OF THE DISCLOSURE

Styryl esters of O,O-di(alkylphenyl) phosphorodithioic acid are provided as antiwear and antioxidant agents for high temperature surfaces in lubricating oils.

#### BACKGROUND OF THE INVENTION

##### Field of the invention

In lubricating oils, particularly ash-free or low ash lubricating oils, used in internal combustion engines, it is common to add antioxidant and antiwear agents. Particularly common additives are the zinc salts of various phosphorodithioic acid esters. However, there have been continual efforts to reduce the amount of metal, as their ions, in lubricating oils. The metals during service frequently enhance deposit formation.

##### Description of the prior art

Numerous patents have issued on the use of phosphorodithioic acid esters in lubricating oils. U.S. Pat. No. 2,528,732 teaches alkyl esters of phosphorodithioic acid. U.S. Pat. No. 2,665,295 teaches the S-terpene ester, while U.S. Pat. No. 2,976,308 teaches an anti-Markownikoff addition of phosphorodithioic acid ester to various olefins, both aromatic and aliphatic. Finally, U.S. Pat. No. 3,352,949 teaches the S- $\alpha$ -phenylethyl ester of dithiophosphoric acid wherein the oxygens are substituted by one alkyl and one alkaryl group.

#### SUMMARY OF THE INVENTION

S- $\alpha$ -phenylethyl O,O-di(alkylphenyl) phosphorodithioates, wherein the alkyl group is of from 10 to 18 carbon atoms, having an average of from 12 to 15 carbon atoms, are used in lubricating oils as antioxidants and antiwear agents, particularly for high temperature service in internal combustion engines, e.g., diesel engines.

#### DESCRIPTION OF THE PREFERRED EMBODIMENTS

The phosphorodithioic acid esters which find use in the lubricating oils of this invention have the following formula:



wherein R is alkyl of from 10 to 18 carbon atoms, having

## 2

an average number of carbon atoms in the range of 12 to 15, preferably a branched chain alkyl, wherein any branch is of from 1 to 2 carbon atoms, preferably 1 carbon atom (methyl), there being at least 1 branch every 4 carbon atoms along the chain;  $\phi$  is phenyl, and Y is hydrogen or lower alkyl of from 1 to 3 carbon atoms, preferably hydrogen or methyl.

Illustrative groups bonded to sulfur are  $\alpha$ -phenylethyl, 2-phenyl-2-propyl, 2-phenyl-2-butyl, etc. Illustrative alkyl groups bonded to the phenyl which is bonded to oxygen are polypropenyl, polyisobutetyl, etc.

The phosphorodithioate esters used in this invention are readily prepared by first preparing the O,O-di-substituted dithiophosphoric acid and reacting the acid at an elevated temperature with the desired olefin. The temperature will generally be in the range of about 50° to 125° C., more usually from 65° to 110° C. The reaction is carried out in the absence of air or other free radical initiator.

- 20 The lubricating oils in which the phosphorodithioic acid esters are used may be derived from natural or synthetic sources. Lubricating oils generally have viscosities of from about 35 to 50,000 Saybolt Universal Seconds (SUS) at 100° F.
- 25 Among natural hydrocarbonaceous oils are paraffinic base, naphthenic base, asphaltic base and mixed base oils. Illustrative synthetic hydrocarbonaceous oils are polymers of various olefins, generally of from 2 to 8 carbon atoms, and alkylated aromatic hydrocarbons.
- 30 The phosphorodithioic acid esters are preferably compounded with from 1 to 15 weight percent of a polyalkylene polyamine lubricating oil detergent. The polyalkylene polyamines will generally have from 2 to 6 nitrogen atoms and alkylene groups of from 2 to 3 atoms.
- 35 Bonded to the alkylene polyamines will generally be from 1 to 2 oil soluble aliphatic hydrocarbon groups, usually a polymer of olefins of from 3 to 4 carbon atoms (propene and isobutylene). The hydrocarbon groups are bonded to the alkylene polyamine directly to nitrogen or through
- 40 a nonoxocarbonyl group such as formyl or succinoyl. The aliphatic hydrocarbon group will generally be of from 30 to 200 carbon atoms, more usually of from 50 to 150 carbon atoms.

Illustrative polyalkylene polyamine detergents are found in U.S. Pats. Nos. 3,219,666, 3,275,554 and 3,087,686.

Other additives may also be present, such as antirust agents, corrosion inhibitors, other detergents, additional oxidation inhibitors, oiliness agents, etc.

- 50 The phosphorodithioic acid esters will generally be present in from 1 to 500 mm./kg. of lubricating oil composition, more usually from about 5 to 50 mm./kg. Above 100 mm./kg., the composition will be as a concentrate for dilution in use.
- 55 The other additives will generally be present individually in from about 0.01 to 15 weight percent, more usually from about 0.05 to 10 weight percent. The alkylene polyamine detergent will usually be present in from 2 to 15 weight percent.
- 60 The following example is offered by way of illustration and not by way of limitation.



## 5

said aliphatic hydrocarbon groups are bonded to nitrogen either directly or through a nonoxocarbonyl group.

5. A lubricating oil composition according to claim 4, wherein said composition of the formula is present in from 1 to 100 mm./kg. of said lubricating oil composition.

6. A lubricating oil composition according to claim 4, wherein said composition of the formula is present in from 1 to 50 mm./kg. of said lubricating oil composition.

## 6

|             |         |                     |          |
|-------------|---------|---------------------|----------|
| 2,657,900   | 11/1953 | Hook et al. -----   | 252—400  |
| 2,665,295   | 1/1954  | Augustine -----     | 252—958  |
| 2,948,682   | 8/1960  | Crosby et al. ----- | 252—46.6 |
| 2,976,308   | 3/1961  | Bacon -----         | 260—978  |
| 3,017,422   | 1/1962  | Thompson -----      | 252—46.6 |
| 5 3,197,496 | 7/1965  | LeSuer -----        | 252—46.6 |
| 3,275,554   | 9/1966  | Wagenaar -----      | 252—50   |

DANIEL E. WYMAN, Primary Examiner

10 J. M. HICKEY, Assistant Examiner

U.S. CL. X.R.

References Cited  
UNITED STATES PATENTS

|           |        |                   |          |
|-----------|--------|-------------------|----------|
| 2,665,295 | 1/1954 | Augustine -----   | 260—958  |
| 2,589,675 | 3/1952 | Cook et al. ----- | 252—46.6 |
| 2,627,523 | 2/1953 | Hook et al. ----- | 252—46.6 |

252—400

UNITED STATES PATENT OFFICE  
CERTIFICATE OF CORRECTION

Patent No. 3,558,490 Dated January 26, 1971

Inventor(s) Warren Lowe

It is certified that error appears in the above-identified patent and that said Letters Patent are hereby corrected as shown below:

Column 1 and Column 4, in the formulae,

S  
|  
P

should read

S  
1  
P

Signed and sealed this 15th day of June 1971.

(SEAL)  
Attest:

EDWARD M. FLETCHER, JR.  
Attesting Officer

WILLIAM E. SCHUYLER, J  
Commissioner of Patent

UNITED STATES PATENT OFFICE  
CERTIFICATE OF CORRECTION

Patent No. 3,558,490 Dated January 26, 1971

Inventor(s) Warren Lowe

It is certified that error appears in the above-identified patent and that said Letters Patent are hereby corrected as shown below:

Column 2, lines 51, 52 and 53, Column 3, Tables I and II, Column 4, Table III, two occurrences and Column 5, lines 5 and 8, "mm./kg.", each occurrence, should read -- mM./kg. --. Column 4, Table IV, "mm.(P)/kg." should read -- mM.(P)/kg. --.

Signed and sealed this 17th day of August 1971.

(SEAL)

Attest:

EDWARD M. FLETCHER, JR.  
Attesting Officer

WILLIAM E. SCHUYLER, JR.  
Commissioner of Patents